

# United States Patent Office

2,735,546

Patented Feb. 21, 1956

1

2,735,546

## THERMAL CONDITIONING FOR ELECTROSTATIC SEPARATION OF GARNET

Foster Fraas, Hyattsville, Md., assignor to the United States of America as represented by the Solicitor of the Department of the Interior

No Drawing. Application December 1, 1952,  
Serial No. 323,524

7 Claims. (Cl. 209—11)

(Granted under Title 35, U. S. Code (1952), sec. 266)

The invention described herein may be manufactured and used by or for the Government of the United States for governmental purposes without the payment to me of any royalty thereon in accordance with the provisions of the act of April 30, 1928 (Ch. 460, 45 Stat. L. 467).

This invention relates to mineral separation and more particularly to the electrostatic separation of garnet from associated minerals.

Garnet found in mineral mixtures is frequently difficult to separate from the other minerals by the common methods of gravity, froth flotation, and magnetic separation. Electrostatic separation may be employed where the more common methods of separation are not practicable. It has been found, however, that many forms of garnet do not possess sufficient electrical conductivity to be selectively separated from nonconductive associated minerals by this method.

Accordingly, an object of this invention is to provide a method for increasing the selectivity of the electrostatic separation of garnet from other minerals.

Another object of this invention is to provide a method for increasing the electrical conductivity of certain forms of garnet whereby the garnet may be selectively separated by electrostatic methods from associated nonconducting mineral.

Another object of this invention is to provide a method whereby certain forms of garnet may be selectively separated from both conductive and nonconductive associated minerals by electrostatic methods.

These and other objects and advantages, hereinafter apparent as the ensuing description proceeds, are accomplished by this invention which comprises thermally conditioning mineral mixtures containing nonconductive forms of garnet to render the garnet conductive prior to the electrostatic separation of garnet from other nonconducting material. An electrostatic separation of this form of garnet from both conducting and nonconducting material may be accomplished by first electrostatically separating the conducting material from the nonconducting fraction, thermally conditioning the nonconducting

2

fraction to render the garnet conductive, and electrostatically separating the garnet from the remaining nonconducting material.

The composition of the garnet group of minerals ranges from garnet theoretically containing only the oxides calcium, magnesium, aluminum, and silicon, such as grossularite  $(\text{CaO})_3 (\frac{1}{2}\text{Al}_2\text{O}_3)_2\text{SiO}_2$  and pyrope  $(\text{MgO})_3 (\frac{1}{2}\text{Al}_2\text{O}_3)_2\text{SiO}_2$ , to garnet in which substantially all of the alkaline earth metal or aluminum, or both alkaline earth metal and aluminum have been replaced by an element of the iron group, namely, Fe, Mn, Cr, or Ni. The presence of an iron group element in the mineral structure contributes to the conducting properties of the mineral. For example, in the complete absence of an iron-group element a conductive structure would not be possible, whereas, in most instances a mineral high in iron-group element content possesses a conductive structure and exhibits the properties of a good conductor upon electrostatic separation.

It has been discovered that many garnet minerals which normally are poor or nonconductors, nevertheless, contain sufficient iron-group elements in such form that they may be converted to conductors by heating to a suitable transition temperature. These garnets include those, such as grossularite,  $(\text{CaO})_3 (\frac{1}{2}\text{Al}_2\text{O}_3)_2\text{SiO}_2$  and pyrope  $(\text{MgO})_3 (\frac{1}{2}\text{Al}_2\text{O}_3)_2\text{SiO}_2$ , for which the theoretical formula indicates no iron group content. Elements of this group do occur, however, in all but the most rare colorless forms of garnet, at least to such an extent that an increase in conductivity takes place upon heat treatment. Other forms of garnet which are rendered more highly conductive upon thermal treatment include rhodolite, uvarovite, and spessartite. While the invention is not to be limited by any theory of chemical or physical transition, it would appear that a crystal change occurs during heating which results in rearrangement of the iron group elements to a form commonly found in semi-conductor crystal structure. That such a change apparently occurs may be noted by visual observation. For example, a garnet before heat treatment may have the transparency of common glass or of quartz or ruby. After heat treatment, and cooling to the original temperature, the garnet is still transparent but has acquired the metallic reflectivity of semi-conductors such as hematite, cuprite, and andradite.

The data of Table I shows the effect of thermal treatment upon a number of mineral varieties of garnet. Almandite and the higher-colored andradites are normally good conductors and require no thermal treatment. Two sources of andradite which are insulators before treatment have no change after treatment. Of the andradites they are the lightest in color and their iron group elements are evidently not available for a conductivity increase after thermal treatment.

Table I.—Thermal conditioning of garnet

| Variety           | Theoretical Formula                                                           | Source                | Color                | Conditioning Effect |       |
|-------------------|-------------------------------------------------------------------------------|-----------------------|----------------------|---------------------|-------|
|                   |                                                                               |                       |                      | Before              | After |
| Rhodolite.....    | $(\text{FeO}, \text{MgO})_3 (\frac{1}{2}\text{Al}_2\text{O}_3)_2\text{SiO}_2$ | Jackson County, N. C. | pink.....            | I                   | C1    |
| Pyrope.....       | $(\text{MgO})_3 (\frac{1}{2}\text{Al}_2\text{O}_3)_2\text{SiO}_2$             | Navajo Res., Ariz.    | bluish red.....      | I                   | C2    |
| Uvarovite.....    | $(\text{CaO})_3 (\frac{1}{2}\text{Cr}_2\text{O}_3)_2\text{SiO}_2$             | Orford, Quebec        | green.....           | I                   | C1    |
| Grossularite..... | $(\text{CaO})_3 (\frac{1}{2}\text{Al}_2\text{O}_3)_2\text{SiO}_2$             | Minas Gerais, Brazil  | brownish red.....    | I                   | C2    |
| Do.....           | $(\text{CaO})_3 (\frac{1}{2}\text{Al}_2\text{O}_3)_2\text{SiO}_2$             | Reddington, Conn.     | grayish orange.....  | I                   | C2    |
| Spessartite.....  | $(\text{MnO})_3 (\frac{1}{2}\text{Al}_2\text{O}_3)_2\text{SiO}_2$             | Madagascar            | orange.....          | I                   | C2    |
| Almandite.....    | $(\text{FeO})_3 (\frac{1}{2}\text{Al}_2\text{O}_3)_2\text{SiO}_2$             | Gore Mtn., N. Y.      | dark red.....        | C1                  |       |
| Andradite.....    | $(\text{CaO})_3 (\frac{1}{2}\text{Fe}_2\text{O}_3)_2\text{SiO}_2$             | Willsboro, N. Y.      | do.....              | C1                  |       |
| Do.....           | $(\text{CaO})_3 (\frac{1}{2}\text{Fe}_2\text{O}_3)_2\text{SiO}_2$             | Ala, Piedmont, Italy  | yellow.....          | I                   |       |
| Do.....           | $(\text{CaO})_3 (\frac{1}{2}\text{Fe}_2\text{O}_3)_2\text{SiO}_2$             | Graham County, Ariz.  | greenish yellow..... | C1                  |       |
| Do.....           | $(\text{CaO})_3 (\frac{1}{2}\text{Fe}_2\text{O}_3)_2\text{SiO}_2$             | Franklin, N. J.       | yellow.....          | I                   | I     |
| Do.....           | $(\text{CaO})_3 (\frac{1}{2}\text{Fe}_2\text{O}_3)_2\text{SiO}_2$             | Oslo, Norway          | black.....           | C1                  |       |

I=insulator; C1=good conductor; C2=poor conductor.

The samples in Table I were conditioned by heating at 650° C. for fifteen minutes, cooling and testing for conductivity. The conductivity test consisted of placing the mineral particle between the terminals of an electrostatic voltmeter of 82 mmf. capacity charged to 280 volts. With minerals designated as insulators, there was no drop in potential during a one minute contact period. With minerals designated as poor conductors, C2, the potential dropped approximately 40 volts in thirty seconds, and with good conductors, C1, much more rapidly. The moisture content of the surrounding air was 34 per cent relative humidity. This is sufficiently low to preclude any surface conductivity due to moisture films. Although heating under reducing conditions may yield higher conductivities, it is a more expensive operation than the above simple procedure of heating in air.

A temperature of about 650° C. is preferred for the thermal treatment. Lower temperatures can be used but the transition rate of the garnet to electrically conductive forms decreases as the temperature is lowered. At 650° C. the transition rate is sufficiently rapid for practical operation. The mineral mixture is then cooled to the customary temperature for electrostatic separation. A temperature between about 20° C. to 100° C. is suitable for this operation.

The electrostatic separation may be secured with any electrostatic separator which separates on the basis of difference in conductance. The dielectrode type of roll separator has been successfully utilized for this purpose.

The invention will be further illustrated by the following examples of practice.

#### EXAMPLE I

This application of the process utilized a North Carolina monazite rich sand containing the commonly associated minerals of garnet, ilmenite and rutile. The garnet was sufficiently low in the iron group elements so as to respond as a nonconductor but had a sufficient content of the iron group elements so as to have the same magnetic susceptibility as the monazite by magnetic methods. The ilmenite and rutile respond as good conductors.

The monazite material was passed through an electrostatic separator. The garnet and monazite collected together as nonconductors while the ilmenite and rutile collected as conductors. The nonconductive fraction, of garnet and monazite, was then given a thermal treatment at about 650° C. for about fifteen minutes. After cooling to room temperature, this fraction was again passed through the electrostatic separator. The garnet now separately collected as a conductor from the monazite as a nonconductor. The results of the separation are summarized in the following tabulation:

Table II.—Effect of thermal conditioning on electrostatic separation

| Product |                         | Conditioning Effect | Weight, Percent | Analysis Geiger count/min. | Distribution Radioactivity, Percent |
|---------|-------------------------|---------------------|-----------------|----------------------------|-------------------------------------|
| No.     | Mineral                 |                     |                 |                            |                                     |
| 1       | rutile-ilmenite, garnet | conductor before.   | 25.4            | 16                         | 0.2                                 |
| 2       |                         | conductor after.    | 36.1            | 13                         | 0.3                                 |
| 3       | monazite                | nonconductor after. | 38.5            | 4,200                      | 99.5                                |
| Total   |                         |                     | 100.0           |                            | 100.0                               |

The ilmenite and rutile fraction collected before the thermal treatment is designated as product 1. The garnet separated as a conductor after thermal treatment is designated as product 2, and the remaining monazite is designated as product 3. It will be seen from the results in Table 2 that the separated products 1 and 2, while making up a substantial part of the total sample on a weight

per cent basis, contained a very small amount of the radioactive monazite. Thus, a highly selective separation has been effected.

#### EXAMPLE II

Monazite sand is deslimed and sized by hydraulic classification to yield two sized fractions, minus 20 plus 35-mesh, and minus 35-mesh. Each fraction is gravity separated on a shaking wet table to remove the quartz as reject. The high density concentrate containing ilmenite, rutile, garnet and monazite is dried at the customary drying temperature of 100 to 150° C. and passed through the electrostatic separator to remove the ilmenite and rutile as conductors from the garnet and monazite as nonconductors.

The garnet and monazite is now heated to the garnet transition temperature. At 650° C. the rate is sufficiently rapid. After cooling the mixture to a temperature below 100° C., the electrostatic separation is repeated to remove the garnet as a conductor from the monazite as a nonconductor. The garnet in this ore was in the form of rhodolite. Rhodolite has a theoretical formula intermediate between pyrope and almandite, part of the MgO in pyrope being replaced by FeO. This particular ore also contained xenotime which separates with the monazite. Xenotime is similar to monazite since it is composed of the rare earth elements. The difference is in the substitution of a small amount of uranium for a small amount of thorium.

The combined results on the minus 20 plus 35-mesh and the minus 35-mesh fractions are summarized in Table III.

Table III.—Gravity and electrostatic concentration of monazite sand

| Product |                                  | Conditioning Effect | Weight, Percent | Analysis Geiger count/min. | Distribution Radioactivity, Percent |
|---------|----------------------------------|---------------------|-----------------|----------------------------|-------------------------------------|
| No.     | Class                            |                     |                 |                            |                                     |
| 1       | rutile-ilmenite, garnet          | conductor before.   | 22.2            | 20                         | 0.3                                 |
| 2       |                                  | conductor after.    | 15.6            | 41                         | 0.4                                 |
| 3       | monazite-xenotime, quartz reject | nonconductor after. | 36.5            | 4,332                      | 97.1                                |
| 4       | 1.                               | -----               | 5.8             | 60                         | 0.2                                 |
| 5       | 2.                               | -----               | 19.9            | 162                        | 2.0                                 |
| Total   |                                  |                     | 100             | 1,628                      | 100                                 |

No complete analysis was made on this ore. The monazite-xenotime fraction by chemical analysis was found to contain 53.7 per cent rare earth oxides. Since monazite and xenotime are the only radioactive minerals in this ore, the Geiger count shows the amount of these minerals in the other fractions. Thus, a highly selective separation has again been made.

In addition to monazite sand, this method may be used wherever a nonconductor fraction occurs in the concentration of garnet ores. Examples are mixtures of diamond and garnet and of kyanite and garnet.

It will be appreciated from a reading of the foregoing specification that the invention herein described is susceptible of various changes and modifications without departing from the spirit and scope thereof.

What is claimed is:

1. A method of conditioning garnet containing an iron-group element and having a mineral form selected from the class consisting of rhodolite, pyrope, uvarovite, grossularite, and spessartite, for electrostatic separation comprising thermally treating said garnet to increase the electrical conductivity thereof.

2. A method of conditioning garnet containing an iron-group element and having a mineral form selected from the class consisting of rhodolite, pyrope, uvarovite, grossularite, and spessartite, for electrostatic separation

comprising heating said minerals to a temperature at which the garnet becomes electrically conductive.

3. A method of conditioning garnet containing an iron-group element and having a mineral form selected from the class consisting of rhodolite, pyrope, uvarovite, grossularite, and spessarite, for electrostatic separation, comprising heating said minerals to a temperature of about 650° C. to increase the electrical conductivity of said garnet.

4. A method for the electrostatic separation of garnet containing an iron-group element and having a mineral form selected from the class consisting of rhodolite, pyrope, uvarovite, grossularite, and spessarite, from associated minerals which respond as nonconductors in the electrostatic process comprising heat-treating said minerals at a temperature at which the garnet becomes electrically conductive, and electrostatically separating the conductive garnet from the nonconductive minerals.

5. A method for the electrostatic separation of garnet containing an iron-group element and having a mineral form selected from the class consisting of rhodolite, pyrope, uvarovite, grossularite, and spessarite, from associated conductive and nonconductive minerals comprising electrostatically separating the conductive minerals from the nonconductive minerals, heating said nonconductive mineral fraction to convert the garnet contained therein to a conductive material, and subjecting the heat-treated material to further electrostatic separative to separate the garnet from the remaining nonconductive material.

6. A method for the separation of garnet from mon-

azite rich sand containing rutile, ilmenite, and garnet containing an iron-group element and having a mineral form selected from the class consisting of rhodolite, pyrope, uvarovite, grossularite, and spessarite, comprising electrostatically separating the rutile and ilmenite from monazite and garnet, heating the monazite-garnet fraction to a temperature of about 650° C., cooling the heated material, and electrostatically separating the garnet from the monazite.

7. A method for the separation of garnet from monazite rich sand containing rutile, ilmenite, and garnet containing an iron-group element and having a mineral form selected from the class consisting of rhodolite, pyrope, uvarovite, grossularite, and spessarite, comprising subjecting said sand to electrostatic separation whereby a conductive fraction containing rutile and ilmenite and a nonconductive fraction containing monazite and garnet are obtained, heat-treating said monazite-garnet fraction at a temperature of about 650° C. to convert the garnet to a conductive form, cooling the heat-treated material to a temperature below 100° C., and subjecting this material to a further electrostatic separation to separate the conductive garnet from the nonconductive monazite.

References Cited in the file of this patent

UNITED STATES PATENTS

|           |                   |               |
|-----------|-------------------|---------------|
| 959,646   | Swart             | May 31, 1910  |
| 1,679,739 | Overstrom         | Aug. 7, 1928  |
| 2,180,804 | Fahrenwald et al. | Nov. 21, 1939 |